

Patented Mar. 5, 1929.

1,704,533

# UNITED STATES PATENT OFFICE.

JUDSON A. DE CEW, OF NEW YORK, N. Y., ASSIGNOR TO PROCESS ENGINEERS, INCORPORATED, OF NEW YORK, N. Y., A CORPORATION OF NEW YORK.

## HYDRATION BY PUMP PRESSURE.

No Drawing.

Application filed April 7, 1926. Serial No. 100,449.

My present invention relates to a paper making machine for hydrating and refining cellulosic fibres.

The principal object of the invention is to hydrate such fibres by causing a rubbing action among themselves, induced by pump pressure.

There are several machines used in paper making that are used for refining the fibres, 10 having a revolving cone or disc rubbing against a stationary surface or one revolving in an opposite direction. The most commonly used machine is the Jordan engine, which is a cone shape machine with a revolving plug. The contact surfaces may be made 15 of abrasive material or they may contain bars or knives.

The paper making material which is to be refined or cut, flows between these rubbing 20 surfaces, while these surfaces are in contact, and a large amount of power is consumed in friction when operating this machine. If the surfaces did not come into contact there would be but little work done on the fibres. I 25 have discovered a method of operating with such machines, which not only reduces greatly the amount of power consumed, but which produces a different action on the pulp fibres, so that a stronger and more pliable sheet of 30 paper can be made.

My method reduces the friction between the rubbing surfaces of the machine and increases the friction between the rubbing surfaces of the fibres, so that the fibres can be 35 hydrated and refined without the fibres being cut by the knives of the machine.

In all Jordans and machines of like character, the pulp is fed to them by gravity, in a 40 fluid condition in which the fibres may be said to be floating or suspended in the water surrounding them. If the pulp stock is not fluid but thickened so that there is no surplus water to suspend the fibres, then the fibres are resting upon other fibres and the stock 45 will not flow by gravity between the rubbing surfaces of the machine.

I have discovered that by the use of pump 50 pressure I can force such a non-liquid fibrous mass between the rubbing surfaces of the Jordan engine or similar machine, and when this is done, a new result is obtained from the use of the machine. The rubbing surfaces are set so that the friction between the surfaces is greatly reduced and the space 55 between these surfaces is filled with a stiff

mass of fibres, which are forced to rub against each other with considerable resistance. An extreme refining and hydrating action is brought to bear, which prepares the stock in a different manner and produces a long pliable fibre that is better for making a strong paper.

The stock may be pumped through the machine and returned to the original tank from which it came, until it has obtained the required character, or it may be forced through a series of machines.

My description of a non-liquid pulp is one from which excess water does not flow readily, the water contained being within and on the surface of the fibres. When the pulp stock has reached the condition that there is no excess water, then there is a marked change in the viscosity of the material.

In forcing the stock through the machine, 75 I may pump it either in the direction of or against the centrifugal force of the machine. By pump pressure, I mean any form of direct pressure, induced by mechanical, hydraulic or pneumatic means, as distinct from a static head. While hydration is the chief object of 80 this invention, a refining of the fibres can also be obtained at the same time.

What I claim as my invention is:—

1. A method of hydrating fibres by means 85 of a Jordan engine, which consists in forcing a non-liquid pulp through the Jordan by means of pump pressure.

2. A method of hydrating paper making fibres, which consists in thickening a mixture 90 of pulp fibres that are dispersed in a water medium, until these fibres are brought into contact with each other, and then forcing them by means of pump pressure through a refining machine of the Jordan type.

3. A method of hydrating pulp fibres, which consists in draining off excess water from the mass until a non-liquid pump is produced and then forcing the mass under 95 pump pressure through a refining engine of the Jordan type.

4. A method of refining pulp fibres, which consists in pumping the pulp through a Jordan engine, without the presence of an aqueous medium suspending the pulp fibres.

5. A method of hydrating pulp fibres in a Jordan engine, which consists in adjusting the revolving surface so that there is no actual contact with the opposing surface, and then forcing the fibres between these surfaces by 110

means of pump pressure, the fibres being in actual contact with each other and not separated by an aqueous medium.

6. A method of hydrating pulp fibres, 5 which consists in forcing the fibres through a Jordan engine by pump pressure, the density of the stock being such that it is non-liquid.

7. A method of hydrating pulp fibres, 10 which consists in pumping the stock through a Jordan engine at such a consistency that there is an insufficient amount of water to float the fibres.

8. A method of hydrating paper pulp fibres by means of a Jordan engine, which 20 consists in bringing the fibres into actual contact with each other, and forcing them through the Jordan at a greater rate than that obtainable under commercial conditions with gravity pressure.

9. A method of hydrating paper making fibres, which consists in moving the stock in a liquid vehicle through a Jordan engine in a pulsating flow.

In testimony whereof, I affix my signature.  
JUDSON A. DE CEW.